



US008293042B2

(12) **United States Patent**  
**Lorentz**

(10) **Patent No.:** **US 8,293,042 B2**  
(45) **Date of Patent:** **Oct. 23, 2012**

(54) **ARTICLES COMPRISING FIBRES AND/OR FIBRIDES, FIBRES AND FIBRIDES AND PROCESS FOR OBTAINING THEM**

(75) Inventor: **Vincent Lorentz**, Bergholtz (FR)

(73) Assignee: **Kermel**, Colmar (FR)

(\*) Notice: Subject to any disclaimer, the term of this patent is extended or adjusted under 35 U.S.C. 154(b) by 0 days.

(21) Appl. No.: **13/156,027**

(22) Filed: **Jun. 8, 2011**

(65) **Prior Publication Data**

US 2012/0001359 A1 Jan. 5, 2012

**Related U.S. Application Data**

(60) Division of application No. 12/195,950, filed on Aug. 21, 2008, now abandoned, which is a continuation of application No. 10/526,676, filed as application No. PCT/FR03/02495 on Aug. 8, 2003, now Pat. No. 7,459,407.

(30) **Foreign Application Priority Data**

Sep. 4, 2002 (FR) ..... 02 10913

(51) **Int. Cl.**

**D04H 1/54** (2012.01)  
**D04H 3/14** (2012.01)

(52) **U.S. Cl.** ..... **156/62.2; 156/181; 156/308.2; 156/309.6; 525/420; 525/537; 525/906**

(58) **Field of Classification Search** ..... **156/62.2, 156/181, 308.2, 309.6; 525/420, 535, 537, 525/906**

See application file for complete search history.

(56) **References Cited**

**U.S. PATENT DOCUMENTS**

|              |         |                  |
|--------------|---------|------------------|
| 3,523,061 A  | 8/1970  | Purvis           |
| 3,534,003 A  | 10/1970 | Hoback et al.    |
| 3,956,561 A  | 5/1976  | Anderson et al.  |
| 3,985,934 A  | 10/1976 | Farrissey et al. |
| 4,552,990 A  | 11/1985 | Persson et al.   |
| 4,703,081 A  | 10/1987 | Blackwell et al. |
| 4,780,359 A  | 10/1988 | Trask et al.     |
| 4,960,549 A  | 10/1990 | Brooks et al.    |
| 5,093,435 A  | 3/1992  | Harris et al.    |
| 5,149,749 A  | 9/1992  | Blackwell et al. |
| 5,164,460 A  | 11/1992 | Yano et al.      |
| 5,173,524 A  | 12/1992 | Satoh            |
| 5,274,875 A  | 1/1994  | Chou             |
| 5,295,406 A  | 3/1994  | Alfano           |
| 6,838,401 B1 | 1/2005  | Murayama et al.  |

**FOREIGN PATENT DOCUMENTS**

|    |                |         |
|----|----------------|---------|
| EP | 648812         | 4/1995  |
| JP | 05-321026 A    | 12/1993 |
| WO | WO 02/12619 A1 | 2/2002  |

**OTHER PUBLICATIONS**

Patent Abstract and Machine Translation for JP 05-321026, Takahiro et al.

Kapantaidakis G C et al. "High Flux Polyethersulfone-Polyimide Blend Hollow Fiber Membranes for Gas Separation" Journal of Membrane Science, Elsevier Scientific Publ. Company, Amsterdam, NL, vol. 204, No. 1-2, Jul. 15, 2002, pp. 153-171.

*Primary Examiner* — Michael Tolin

(74) *Attorney, Agent, or Firm* — Millen, White, Zelano & Branigan, P.C.

(57) **ABSTRACT**

The present invention relates to novel articles, especially non-woven articles comprising fibers and/or fibrils. It also relates to novel fibers and fibrils and to a process for obtaining these fibers and fibrils.

**22 Claims, 1 Drawing Sheet**





Figure 1



Figure 2

**ARTICLES COMPRISING FIBRES AND/OR  
FIBRIDS, FIBRES AND FIBRIDS AND  
PROCESS FOR OBTAINING THEM**

This application is a divisional application of parent application Ser. No. 12/195,950 filed Aug. 21, 2008, now abandoned which is a continuation of application Ser. No. 10/526,676 filed Mar. 4, 2005 now U.S. Pat. No. 7,459,407, which is a National Stage Application of PCT International application PCT/FR03/02495 filed Aug. 8, 2003, and claiming priority of French application 0210913 filed Sep. 4, 2002, all of said applications being incorporated by reference herein.

The present invention relates to novel articles, especially non-woven articles comprising fibres and/or fibrids. It also relates to novel fibres and fibrids and to a process for obtaining these fibres and fibrids.

Particularly in the electrical insulation field, the aim is to obtain products exhibiting good temperature resistance and good mechanical properties and/or dielectric properties. These products may, for example, be non-woven articles produced from thermally stable fibres. In such an article, good cohesion of the thermally stable fibres is necessary for obtaining a good level of mechanical properties, or indeed also a uniform and dense structure of the article in order to obtain dielectric properties. For this purpose, the aim is to obtain good cohesion of the thermally stable fibres within the article. The aim is also to obtain a uniform and compact structure within the article. These articles, depending on their structure (especially their density) and/or their formulation, may have a mechanical and/or dielectric reinforcement function.

Document U.S. Pat. No. 2,999,788 proposes, for example, the preparation of synthetic polymer particles or "fibrids" having a particular structure, that can be used with fibres based on synthetic polymers, for the production of coherent fibrous structures by a papermaking process. A hot-pressing operation may be carried out on these structures, causing the fibrids to undergo plastic flow. However, the preparation of such fibrids, carried out by precipitation in a sheared medium, is complicated and expensive. These fibres must also remain in aqueous medium in order to be used directly. Consequently, they can neither be isolated nor transported easily, which limits their use.

Document FR 2 163 383 proposes to prepare non-woven articles formed by a web of fibres based on a non-melting material or one having a melting point above 180° C., the fibres being bonded together by means of a polyamide-imide bonding agent used in a proportion of 5 to 150% of the weight of dry fibres employed. However, the impregnation with resin is carried out in solution in a solvent, which consequently has deleterious effects on the characteristics of the non-wovens.

To improve the feasibility of non-woven webs, document FR 2 156 452 proposes to prepare non-woven webs by a wet route, the webs being formed from fibres made of a non-melting material or one having a melting point above 180° C., bonded together by a thermoplastic polymer in powder form.

Although in theory these webs can be obtained by a papermaking technique, industrial production of such webs is in fact difficult: this is because the compound comprising synthetic fibres and resin-based bonding agent has too low a cohesion to be able to be handled and in particular such a compound has insufficient cohesion to be able to be prepared dynamically, for example on a commercial papermaking machine; such webs are mainly able to be produced on laboratory apparatuses of the "Formette Franck" type, that is to say in a static and batch manner, as is apparent from the examples.

Document FR 2 685 363 proposes the wet preparation of a paper formed from fibres, having a thermal endurance at greater than or equal to 180° C., the fibres being bonded together by means of a fibrous bonding agent and a chemical bonding agent.

The use of bonding agents for ensuring fibre cohesion in articles, for example non-woven articles in particular, poses difficulties and incurs costs as regards the use of these bonding agents.

The present invention provides novel articles, especially non-woven articles, not having the above drawbacks, comprising fibres and/or fibrids. The invention also provides novel fibres and fibrids, and a process for obtaining these fibres and fibrids, and articles obtained from these fibres and fibrids, such as non-woven articles. The thermoplastic part of the fibre or fibril of the invention acts in particular as the chemical bonding agent described above. In particular, it has the property of "undergoing plastic flow" under a compressive stress and temperature stress. This thus ensures the cohesion of the thermally stable fibres in these articles and their level of thermal and mechanical properties is very satisfactory. These articles may have a dense uniform structure, and therefore a good level of dielectric properties.

For this purpose, the first subject of the invention is an article comprising at least fibres and/or fibrids, characterized in that the fibres and fibrids are formed from a polymer blend comprising at least:

30 A thermally stable polymer; and  
A thermoplastic polymer chosen from the group of polysulphides and polysulphones.

The second subject of the invention is a fibre and a fibril such as those described above and a process for obtaining them.

35 In a third subject, the invention proposes the use of the articles as described above in the field of electrical insulation.

The thermally stable polymer of the invention is preferably a non-melting polymer or one having a glass transition temperature above 180° C., preferably greater than or equal to 230° C., or higher. The thermally stable polymer of the invention has a long-term thermal withstand (that is to say capability of retaining in particular its physical properties) at a temperature above 180° C. This thermally stable polymer is 40 preferably chosen from polyaramids and polyimides. Mention may be made, as examples of polyaramids, of aromatic polyaramides, such as the polymer known by the brand name Nomex®, or polyamide-imides, such as the polymer known by the brand name Kermel®. As an example of polyimides, mention may be made of the polyimides obtained according to document EP 0 119 185, known by the brand name P84®. The aromatic polyaramides may be as described in Patent EP 0 360 707. They may be obtained using the process described in Patent EP 0 360 707.

45 The thermoplastic polymer is chosen from the group of polysulphides and polysulphones. As an example of a polysulphide, mention may be made of polyphenylene sulphide denoted hereafter by PPS. As an example of polysulphones, denoted hereafter by PSU, mention may be made of polyethersulphone denoted hereafter by PESU or polyphenylene sulphone denoted hereafter by PPSU.

50 These thermoplastic polymers have a glass transition temperature of less than or equal to 250° C., thereby allowing them to act in particular as a chemical bonding agent in the articles of the invention and allowing them to undergo "plastic flow" under a compressive stress and temperature stress.

These polymers also have good thermal stability, since they belong to a thermal class (thermal index) above 130° C. This is advantageous for obtaining articles exhibiting good thermal stability.

According to a preferred embodiment of the invention, the thermoplastic polymer and the thermally stable polymer are soluble in the same solvent. Advantageously, the solvent is an aprotic polar solvent. It is more preferably chosen from DMEU, DMAc, NMP and DMF.

Advantageously, the fibre or fibrid according to the invention comprises at least 10% by weight of thermoplastic polymer.

Fibrids are small non-granular fibrous particles or particles in the form of films that are not rigid. Two of their three dimensions are of the order of a few microns. Their small size and their flexibility allow them to be deposited in physically interlaced configurations, such as those commonly found in papers formed from pulp.

The fibre according to the invention preferably has a linear density of between 0.5 dtex and 13.2 dtex. The fibre of the invention preferably has a length of between 1 and 100 mm.

The fibre according to the invention may have varied cross-sectional shapes, such as a round, trilobate or "flat" shape. The term "fibre of flat cross-sectional shape" is understood to mean a fibre whose length/width ratio is greater than or equal to 2.

The fibre or fibrid according to the invention may be treated with a size.

According to one particular embodiment of the article of the invention, the fibres are obtained by blending the thermally stable polymer with the thermoplastic polymer, followed by spinning the blend.

Any means known to those skilled in the art for blending two polymers may be used. Preferably, the polymers are blended by dissolving the polymers in at least one common solvent. The thermoplastic polymer and the thermally stable polymer may be dissolved together, simultaneously or in succession, in a solvent or a mixture of mutually miscible solvents, for example in a single reactor. The polymers may also be dissolved separately in the same solvent or in different solvents that are mutually miscible, for example in two different containers, and then the polymer solutions are mixed together.

The dissolution conditions, such as the temperature, are determined by those skilled in the art according to the nature of the polymers and the solvent(s) that is (are) used. The dissolution may, for example, be carried out hot, with stirring, in order to facilitate the dissolution.

The dissolution may be carried out at room temperature. Preferably, the dissolution temperature is between 50 and 150° C.

The dissolving solvent(s) is (are) advantageously aprotic polar solvents. It is possible to use a dimethylalkylene urea, for example dimethylethylene urea (DMEU) or dimethylpropylene urea. Preferably, it is chosen from DMEU, dimethylacetamide (DMAc), N-methylpyrrolidone (NMP) and dimethylformamide (DMF). The dissolving solvent may be a mixture of aprotic polar solvents, for example a mixture of dimethylethylene urea and an anhydrous aprotic polar solvent, such as NMP, DMAc, DMF, tetramethyl urea or  $\gamma$ -butyrolactone.

The polymer solution obtained after dissolution is called colloidion. The solution obtained is preferably clear.

The total concentration by weight of the polymers relative to the solution is preferably between 5 and 40%.

The solution may also include additives, such as pigments, reinforcing agents, stabilizers and delustrants.

The solution must also have a viscosity allowing it to be spun, generally between 100 and 1000 poise. For wet spinning, the viscosity is preferably between 400 and 800 poise, measured by means of a viscometer known by the brand name EPPRECHT RHEOMAT 15. For dry spinning, the viscosity is preferably between 1500 and 3000 poise.

The polymer blend may also be produced in-line during the spinning step, for example by the in-line injection of each polymer, whether or not dissolved in a solvent, during the spinning process.

Any method of spinning a polymer blend, especially a polymer solution, known to those skilled in the art may be used here within the context of the invention.

Mention may be made, for example, of dry spinning, in which the polymer solution (fibre-forming substance in the dissolved state) is extruded through capillaries in an environment favourable for the removal of the solvent, for example in an evaporating atmosphere maintained at a temperature close to or above the boiling point of the solvent, allowing the filaments to solidify. The filaments leaving the evaporating chamber are stripped of their residual solvent. To do this, they may be washed with water, optionally boiling water under pressure, and then they are usually dried, preferably at a temperature above 80° C. They may also be heat-treated at a temperature greater than or equal to 160° C. under reduced pressure and/or in an inert atmosphere. After having been stripped of their residual solvent, they may be drawn, for example at a temperature above 250° C., preferably greater than 300° C., preferably in the absence of oxygen.

According to one particular embodiment of the invention, the spinning method is a wet spinning method, in which the polymer solution (solution of fibre-forming substances) is extruded into a coagulating bath.

The temperature of the spinning solution may vary widely, depending on the viscosity of the solution to be spun. For example, a solution having a low viscosity may be easily extruded at ordinary temperatures, whereas for a solution having a high viscosity, it is preferable for this to be extruded hot, for example at 120° C. or even higher, so as to avoid excessively high pressures in the die. The spinning solution is advantageously maintained between 15 and 40° C., preferably between 15 and 25° C.

The coagulating bath used in the process according to the invention is preferably an aqueous solution containing from 30 to 80% by weight, preferably from 40 to 70% by weight, of a solvent or solvent mixture, preferably a dimethylalkylene urea (DMAU) or DMF, or a mixture thereof, although it is often advantageous to use a bath containing more than 50% by weight of solvent in order to obtain filaments having better drawability, and therefore better final properties.

Preferably, the polymers of the solution to be spun have similar coagulation rates.

The spinning rate in the coagulating bath may vary widely, depending on its solvent concentration and the distance that the filaments travel through this bath. This spinning rate in the coagulating bath may be readily chosen to be between, for example, 10 and 60 m/min, although higher rates can be achieved. It is generally not advantageous to spin at lower rates for process efficiency reasons. Moreover, excessively high spinning rates in the coagulating bath reduce the drawability of the filaments in air. The spinning rate in the coagulating bath will therefore be chosen to take into account both the efficiency and the desired properties of the finished filament.

The filaments leaving the coagulating bath in the gel state are then drawn, for example in air, with a draw ratio defined by  $(V_2/V_1) \times 100$ ,  $V_2$  being the velocity of the drawing rolls

and  $V_1$  that of the feed rolls. The draw ratio of the yarns in the gel state is greater than 100%, preferably greater than or equal to 110% or even higher, for example greater than or equal to 200%.

After drawing, preferably in air, generally carried out by passage between two series of rolls, the residual solvent is removed from the filaments by known means, generally by means of a washing operation using water flowing counter-currently, or on washing rolls, preferably at room temperature.

According to another particular embodiment of the invention, the spinning method is a dry spinning method.

In the two spinning processes described above (dry spinning and wet spinning), the washed filaments are then dried by known means, for example in a dryer or over rolls. The temperature of this drying may vary widely, as may the drying rate, which is higher the higher the temperature. It is generally advantageous to carry out drying with a progressive rise in the temperature, this temperature possibly reaching and even exceeding 200° C. for example.

The filaments may then undergo hot overdrawing, in order to improve their mechanical properties and in particular their tenacity, which may be beneficial for some applications.

This hot overdrawing may be carried out by any known means: oven, plate, roll, roll and plate, preferably in a closed chamber. It is carried out at a temperature of at least 150° C., possibly a temperature of up to or even exceeding 200 to 300° C. The overdraw ratio is generally at least 150%, but it may vary widely depending on the desired properties of the finished yarn. The total draw ratio is therefore at least 250%, preferably at least 260%.

The combination of drawing and possibly overdrawing may be carried out in one or more stages, continuously or batchwise, with the above operations. Furthermore, the overdrawing may be combined with drying. To do this, all that is required is to provide, at the end of drying, a higher temperature zone for the overdrawing.

The filaments obtained are then chopped into fibres using a method known to those skilled in the art.

According to another embodiment of the article of the invention the fibrils are obtained by blending the thermally stable polymer with the thermoplastic polymer, followed by precipitation of the blend under a shear stress.

The thermally stable polymer/thermoplastic polymer blend may be produced in a manner similar to that described above for the fibres.

The fibrils of the invention may especially be obtained by precipitating a polymer solution in a fibrilizing apparatus of the type described in U.S. Pat. No. 3,018,091, in which the polymers are sheared while they are precipitating.

According to a particular embodiment of the invention, the articles are non-woven articles. The non-woven articles are in the form of sheets, films or felts, and in general they define any coherent fibrous structure not involving any textile operation, such as spinning, knitting or weaving.

The article may be obtained from a single type of fibre or on the contrary from blends of fibres. The non-woven article of the invention comprises, at least in part, fibres and/or fibrils according to the invention. The article of the invention may comprise fibres of different kinds and/or fibrils of different kinds. Apart from the fibres and/or fibrils according to the invention, the non-woven article may comprise, for example, thermally stable or reinforcing fibres and/or fibrils of the para-aramid type, meta-aramid type, polyamide-imide type, etc.

The non-woven article may comprise, for example, fibres according to the invention and thermally stable fibres. If the

article comprises fibrils, the article may, for example, comprise fibres according to the invention and fibrils of thermally stable polymer according to a first embodiment; or the article, may, for example, comprise thermally stable fibres and fibrils according to the invention according to another embodiment.

The non-woven article of the invention may be obtained by a method and an apparatus for preparing a non-woven article that are known to those skilled in the art. The article of the invention is generally obtained by carrying out a "web-forming" step, that is to say a step in which the fibres and/or fibrils are spread out over a surface, followed by a step of "consolidating" the structure obtained.

According to an advantageous embodiment of the invention, the "web-forming" step is carried out "dry" ("drylaid" process), for example starting in particular with fibres of the invention having a length of between 40 and 80 mm. The fibres may, for example, be treated using an ordinary carding machine.

According to another advantageous embodiment of the invention, the "web-forming" step is carried out "wet" or by "papermaking means" ("wetlaid" process). The fibres used in this embodiment generally have a length of between 2 and 12 mm, preferably between 3 and 7 mm, and their linear density, expressed in decitex, is generally between 0.5 and 20. Theoretically, it is possible to use fibres having a length greater than 12 mm, but in practice longer fibres entangle, requiring a larger amount of water, thereby making the process more expensive and more complicated.

According to this embodiment, the non-woven article is obtained by introducing the various constituents of the article into the water, namely the fibres and a fibrous bonding agent composed of a pulp based on a synthetic polymer having a thermal endurance at greater than or equal to 180° C. (such as a para-aramid pulp) and/or fibrils based on a synthetic polymer having a thermal endurance at greater than or equal to 180° C. and/or fibrils according to the invention, and optionally other desirable adjuvants, additives or fillers.

The pulp based on a synthetic polymer possessing a thermal withstand greater than or equal to 180° C. is generally obtained from fibres of usual length, especially fibrils, in a manner known per se, in order to give it a large number of catching points and thus increase its specific surface area. Among synthetic fibres, only highly crystallized fibres may be fibrillized. This is the case with completely aromatic polyamides and polyesters, but other highly crystallized polymers are able to be split along the fibre axis or are fibrillizable.

To improve certain properties, adjuvants, additives or fillers may also be used in various proportions depending on the desired properties; for example, mica may be introduced in order to further increase the dielectric properties of the article.

The "papermaking method" of preparing non-woven articles is known to those skilled in the art.

The step of "consolidation" of the structure obtained by web forming, as described above, may be carried out according to any method known to those skilled in the art. Preferably, the "consolidation" is carried out thermally, for example by thermal pressing of the article. The thermal pressing temperature is generally greater than the glass transition temperature of the thermoplastic polymer of the fibres and/or fibrils according to the invention contained in the article. Preferably, the thermal pressing temperature is between the glass transition temperature and the softening temperature of the thermoplastic polymer.

According to one advantageous embodiment of the invention, the thermal pressing temperature is between 200 and 350° C. Preferably, the pressure is greater than or equal to 5 bar.

This pressing densifies and consolidates the article of the invention. It is generally accompanied by plastic flow of the thermoplastic polymer of the fibres and/or fibrils according to the invention contained in the article through the structure of the article.

There is no limitation imposed as to the way in which the thermal pressing is carried out. Any means of thermally pressing a non-woven article may be used.

For example, the pressing may be carried out using a press or a calender with heated rolls. It is possible to carry out several passes on the pressing apparatus so as to obtain the desired density.

The preferred thermal pressing method of the invention is calendering.

According to a particular embodiment of the invention, the thermal pressing is carried out using a continuous press.

The articles obtained by this pressing are various and varied depending on the thermal pressing conditions employed—especially the pressing temperature, pressure and time—and depending on the formulation of the article—especially the amount of fibres and/or fibrils according to the invention contained in the article and the amount of thermoplastic polymer present in these fibres and/or fibrils.

These parameters are chosen according to the type of article and the desired properties of this article.

The articles of the invention may be used especially in the electrical insulation field.

The role of the articles varies depending on their density and therefore on their strength/dielectric properties. They may for example, be used in an insulation system, in which the main, insulant is an oil or a resin, as a mechanical “spacer” or “reinforcement” to be inserted between two parts to be electrically isolated. The articles may also be used directly as insulant in insulation systems of the “dry” type.

The invention also relates to a fibre characterized in that it is formed from a polymer blend comprising at least:

A thermally stable polymer; and  
A thermoplastic polymer chosen from the group of polysulphides and polysulphones;  
and in that it has a linear density of less than or equal to 13.2 dtex.

The invention also relates to a fibrid, characterized in that it is formed from a polymer blend comprising at least:

A thermally stable polymer; and  
A thermoplastic polymer chosen from the group of polysulphides and polysulphones.

Everything described relating to the thermally stable polymer, the thermoplastic polymer, the fibres and fibrils of the articles of the invention, the process for obtaining the fibres and the process for obtaining the fibrils applies here in the same way for the fibres and fibrils of the invention above.

The invention also relates, in a third subject, to the use of the articles of the invention as described above in the electrical insulation field.

Further details and advantages of the invention will become more clearly apparent in the light of the examples described below.

## EXAMPLES

### Examples 1 to 3

#### Preparation of the Thermoplastic Polymer/Thermally Stable Polymer Blend

##### Example 1

180 kg of DMEU solvent were introduced into a heated and stirred reactor. This solvent was firstly heated to a temperature

of between 60° C. and 120° C. The PESU polymer (MW: 80 000 to 90 000 g/mol) in the form of lenticular granules was introduced into the hot solvent, in ten equal fractions. The time required between each fraction depended on the intensity of the stirring and the temperature. The polymer was introduced until it represented 20 to 40% by weight of the blend.

The polymer content in the solution influences its viscosity. As an example, at 21% the viscosity at 25° C. is 350 poise; at 28% the viscosity is 460 poise.

The PESU thermoplastic polymer was blended with the Kermel® polyamide-imide by melt blending, between 60 and 120° C., the blend described above containing the PESU and a 21 wt % solution of Kermel® polyimide-inside in the DMEU solvent (MW: 150 000 g/mol (polystyrene equivalent); viscosity: 600 poise at 25° C.). The proportion of the two solutions in the blend was expressed as the proportion of PESU polymer in the dry matter and was between 40 and 60%.

### Example 2

A Kermel® polyamide-imide/PESU blend was obtained directly by dissolving the PESU polymer in a 13 wt % solution of Kermel® polyamide-imide in the DMEU solvent using a blender having a high shear rate and a high degree of recycling.

### Example 3

A mixture containing the PESU was prepared according to the operating method of Example 1. The blend with the Kermel® polyamide-imide (in the form of a 21 wt % solution of Kermel® polyamide-imide in the DMEU solvent) was produced during the spinning, by conjointly injecting the two solutions into a common line, upstream of the static mixers installed in this line, which feeds the spinning unit. The proportions of the two solutions in the blend is respected by adjusting the rotation speeds of metering pumps.

### Examples 4 and 5

#### Spinning of Thermoplastic Polymer/Thermally Stable Polymer Blends

##### Example 4

The PESU/Kermel® polyimide-imide blends of Examples 1 to 3 were spun using a wet spinning process. The proportion of PESU polymer was 40% by weight. The conditions below represent, as examples, the spinning parameters used:

Dies: 10 000 holes 50 µm in diameter  
Coagulation bath: 55% solvent, 19° C.  
Spinning rate: 14 m/min  
Draw ratio: 2x  
Final linear density obtained: 4.4 dtex.  
The fibre was dried, crimped and chopped conventionally (fibre length: 60 mm).

##### Example 5

The PESU/Kermel® polyamide-imide blends of Examples 1 to 3 were spun using a wet spinning process. The proportion of PESU polymer was 50%. The conditions below represent, as examples, the spinning parameters used:

Dies: 10 000 holes 40 µm in diameter  
Coagulation bath: 60% solvent, 19° C.

Spinning rate: 14 m/min

Draw ratio: 2x

Final linear density obtained: 2.2 dtex.

The fibre was dried conventionally. The crimping and chopping were carried out conventionally.

Examples 6 to 8

#### Articles

Non-woven articles of various grammages were prepared from the fibres of Example 4 using the "dry method" and by "consolidation" (carding, web forming, calendering) according to a method known to those skilled in the art.

The equipment employed was the following:

parallel-output Garnett®-type carding machine;

Asselin® web former;

KTM® calender.

Table 1 describes the operating conditions used and the characteristics of the articles obtained. The mechanical properties—strength and elongation at break—were measured according to the NF-EN 29073-3 standard of December 1992. The thickness of the articles was measured using a Palmer®-type micrometer.

TABLE 1

|                                             | Examples  |               |           |
|---------------------------------------------|-----------|---------------|-----------|
|                                             | Example 6 | Example 7 (*) | Example 8 |
| Calendering rate (m/min)                    | 5         | 5             | 5         |
| Calendering temperature (° C.)              | 250       | 250           | 270       |
| Calendering pressure (bar)                  | 6         | 6             | 6         |
| Grammage (g/m <sup>2</sup> )                | 42        | 60            | 65        |
| Thickness (μm)                              | 50        | 65            | 70        |
| Density (g/cm <sup>3</sup> )                | 0.84      | 0.92          | 0.93      |
| Machine direction tensile strength (N/5 cm) | 20.2      | 41            | 60.9      |
| Machine direction elongation at break (%)   | 1.4       | 2.1           | 2.9       |

(\*) the article according to Example 7 was subjected to two calendering passes.

The plastic flow and the density obtained after calendering were observed.

FIG. 1 is a photograph of the surface of the article according to Example 8 after calendering.

FIG. 2 is a photograph of the cross section of the article according to Example 8 after calendering.

Examples 9 to 12

#### Preparation of Fibrids from a Thermoplastic Polymer/Thermally Stable Polymer Blend

The PESU/Kermel® polyamide-imide blend of Example 1, diluted with DMEU in order to obtain the desired concen-

tration of PESU/Kermel® polyamide-imide polymers, was precipitated under high shear using a method as described in the documents FR 1214 126 or U.S. Pat. No. 4,187,143, in an aqueous coagulation bath having a given concentration of DMEU solvent. Table 2 gives the conditions for preparing the fibrids.

TABLE 2

| Examples | Proportion of PESU/Kermel® polyamide-imide by weight (%) before precipitation |    | Proportion of the solvent in the coagulation bath by weight (%) |
|----------|-------------------------------------------------------------------------------|----|-----------------------------------------------------------------|
|          | 9                                                                             | 15 |                                                                 |
| 10       | 9.5                                                                           | 25 |                                                                 |
| 11       | 15                                                                            | 50 |                                                                 |
| 12       | 9.5                                                                           | 0  |                                                                 |
|          |                                                                               |    | 50                                                              |

The characteristics of the fibrids were measured on the MORFI apparatus (conventional apparatus for measuring papermaking cellulose fibres). Table 3 gives these characteristics.

TABLE 3

|                                     | Examples |       |       |       |
|-------------------------------------|----------|-------|-------|-------|
|                                     | 9        | 10    | 11    | 12    |
| Length (mm)                         | 0.315    | 0.431 | 0.351 | 0.289 |
| Width (μm)                          | 40.2     | 44.6  | 49.7  | 30.3  |
| Fine elements (%) by length         | 19.5     | 11.0  | 14.7  | 24.9  |
| Amount of fine elements (%) by area | 1.6      | 0.4   | 0.6   | 3.6   |

Examples 13 to 16

#### Articles Obtained from Fibrids

The fibrids of Examples 9 to 12 were blended with an equal weight of Kermel® polyamide-imide fibres 6 mm in length. These four preparations were used to produce papers on a Frank-type handsheet apparatus by wet processing and according to a conventional papermaking process. The intended weight of the specimens was 80 g/m<sup>2</sup>. The characteristics of the papers are given in Table 4.

The retention factor was defined as follows:

$$\text{Retention factor (\%)} = (1 - \frac{\text{mass introduced (g)} - \text{mass after passing through (g)}}{\text{mass introduced (g)}}) \times 100.$$

TABLE 4

| Examples | Fibrids | Thickness in μm | Mass introduced into the apparatus (g) | Mass after passing through the apparatus (g) | Retention factor (%) | Grammage (g/m <sup>2</sup> ) | Hand (cm <sup>3</sup> /g) |
|----------|---------|-----------------|----------------------------------------|----------------------------------------------|----------------------|------------------------------|---------------------------|
|          |         |                 | (g)                                    | (g)                                          |                      |                              |                           |
| 13       | Ex. 9   | 199.6           | 2.506                                  | 2.448                                        | 98                   | 77                           | 2.6                       |
| 14       | Ex. 10  | 238.8           | 2.516                                  | 2.478                                        | 98                   | 81                           | 2.9                       |

TABLE 4-continued

| Examples | Fibrils | Thickness in $\mu\text{m}$ | Mass introduced into the apparatus (g) | Mass after passing through the apparatus (g) | Retention factor (%) | Grammage age (g/ $\text{m}^2$ ) | Hand ( $\text{cm}^3/\text{g}$ ) |
|----------|---------|----------------------------|----------------------------------------|----------------------------------------------|----------------------|---------------------------------|---------------------------------|
| 15       | Ex. 11  | 199.5                      | 2.517                                  | 2.342                                        | 93                   | 74                              | 2.7                             |
| 16       | Ex. 12  | 191.3                      | 2.525                                  | 2.500                                        | 99                   | 77                              | 2.5                             |

After drying, the papers obtained were characterized by their mechanical properties (Table 5) and by their air permeability in the Bendtsen apparatus at a pressure of 1.47 kPa (Table 6) using the conventional methods of the papermaking industry.

TABLE 5

| Mechanical strength of the papers |          |      |      |      |
|-----------------------------------|----------|------|------|------|
|                                   | Examples |      |      |      |
|                                   | 13       | 14   | 15   | 16   |
| Breaking force (N)                | 1.78     | 2.37 | 1.05 | 3.23 |
| Tensile strength (N/m)            | 119      | 158  | 70   | 216  |
| Tensile strength index (Nm/g)     | 1.55     | 1.95 | 0.94 | 2.84 |
| Elongation at break (%)           | 1.89     | 2.61 | 1.16 | 2.09 |
| Elastic modulus (MPa)             | 558      | 370  | 638  | 632  |
| Tear strength (mN)                | 820      | 1600 | 560  | 1400 |
| Tear Index (Nm/g)                 | 3.27     | 6.07 | 2.32 | 5.6  |

TABLE 6

| Air permeability   |          |      |       |     |
|--------------------|----------|------|-------|-----|
|                    | Examples |      |       |     |
|                    | 13       | 14   | 15    | 16  |
| Mean (ml/min)      | 50.5     | 58.7 | 876.8 | 1.4 |
| Standard deviation |          | 4.9  | 124.9 | 0.2 |

Examples 17 to 24

## Hot-Pressed Articles Obtained Fibrils

The papers of Examples 13 to 16 were hot-pressed in a laboratory platen press at 280° C.:  
either for 10 min at 100 bar  
or for 5 min at 200 bar.

TABLE 7

| Thickness of the pressed papers |                        |              |              |              |              |
|---------------------------------|------------------------|--------------|--------------|--------------|--------------|
|                                 | Examples               |              |              |              |              |
|                                 | 17                     | 18           | 19           | 20           |              |
| Pressure: 100 bar               | Article Mean thickness | Ex. 13 125.8 | Ex. 14 137.3 | Ex. 15 125.7 | Ex. 16 121.5 |

TABLE 7-continued

| Thickness of the pressed papers |                                                   |      |      |      |      |
|---------------------------------|---------------------------------------------------|------|------|------|------|
|                                 | ( $\mu\text{m}$ ) Hand ( $\text{cm}^3/\text{g}$ ) | 1.63 | 1.69 | 1.69 | 1.57 |
| Examples                        |                                                   | 21   | 22   | 23   | 24   |

15 The invention claimed is:  
1. A method for preparing a consolidated dense and substantially uniform article, wherein the article comprises thermostable fibers and/or fibrils formed from a blend of polymers comprising at least one thermostable polymer having a glass transition temperature greater than or equal to 230° C. and a thermoplastic polymer having a glass transition temperature of less than or equal to 250° C., said thermoplastic polymer being at least one polysulfide or at least one polysulfone, said method comprising forming an unwoven web of said fibers and/or fibrils and consolidating said web, said consolidating comprising heat pressing said web at a temperature above the glass transition temperature of said thermoplastic polymer, said thermoplastic polymer acting as a chemical bonding agent in said article to ensure cohesion of the thermostable fibers and/or fibrils.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070

## 13

12. A method according to claim 1, wherein the article comprises said fibrils and said fibrils are obtained by mixing the thermostable polymer and the thermoplastic polymer and then shear precipitating the mixture.

13. A method according to claim 1, wherein the heat pressing is performed at pressure and temperature conditions that impart plastic flow to at least the thermoplastic polymer.

14. A method according to claim 1, wherein during heat pressing, the temperature is in the range of 200° C. to 350° C., and the pressure is 5 bars or more.

15. A method according to claim 1, wherein the article further comprises additional fibers and/or fibrils which are thermostable.

16. A method according to claim 1, wherein the fibers have a size of 13.2 dtex or less.

17. A method according to claim 1, wherein the article is electrical insulation.

## 14

18. A method according to claim 1, wherein the thermostable fibers and/or fibrils are para-aramid, meta-aramid or polyamide imide fibers.

19. A method according to claim 1, wherein the consolidated fiber-based dense and substantially uniform article is free of mica.

20. A method according to claim 1, wherein the thermoplastic polymer is polyether sulfone or polyphenylene sulfone and the thermostable fibers and/or fibrils are para-aramid, meta-aramid or polyamide imide fibers.

21. A method according to claim 1, wherein said steps of forming an unwoven web and consolidating comprises carding, web forming and calendering.

22. A method according to claim 1, wherein said thermoplastic polymer is at least one polysulfide.

\* \* \* \* \*